

# UNITED STATES PATENT OFFICE.

HANS GOLDSCHMIDT AND KARL MÜLLER, OF ESSEN, GERMANY, ASSIGNEES, BY MESNE ASSIGNMENTS, TO THE CHEMICAL FOUNDATION, INC., A CORPORATION OF DELAWARE.

## ZINC ALLOY.

1,338,826.

Specification of Letters Patent.

Patented May 4, 1920.

No Drawing.

Application filed April 19, 1917. Serial No. 163,263.

To all whom it may concern:

Be it known that we, HANS GOLDSCHMIDT and KARL MÜLLER, doctors of chemistry, citizens of the German Empire, residing at 5 Essen, Province of the Rhine, Germany, Salkenbergsweg 18, have invented a new and useful Improvement in Zinc Alloys; and we do hereby declare the following to be a full, clear, and exact description of the 10 same.

In recent times it has been tried to replace white-metal for bearings as well as red-brass by alloys which contain besides zinc in the main more or less tin (up to 20 15 per cent.) and small amounts of copper, lead and aluminum.

Our invention refers to zinc alloys free of tin which can be used as a substitute for the above named metals. It has been found 20 that for the purpose mentioned zinc alloys are useful which contain about 90 per cent. of zinc and copper, lead and aluminum in varying proportions without any addition of tin. Moreover we have found that by 25 adding manganese as a further constituent alloys are obtainable which can be cast and worked without any difficulty and which owing to their favorable mechanical properties are eminently useful for bearings, fittings, fuses and the like. Of special value 30 in practice has proved an alloy containing about 6 per cent. of copper, 2 per cent. of aluminum and 1.5 per cent. of manganese besides zinc.

35 Of course the proportions of the com-

ponent parts may be varied within certain limits, in practical use it is preferred adding not more than 4 per cent. and not less than 0.25 per cent. of manganese.

A characteristic feature of this new alloy 40 is that it is without any tin and furthermore that it contains a small amount of manganese.

What we claim is:

1. An alloy containing zinc, and from 45 about one-quarter of one (.25) per cent. to about four (4) per cent. of manganese, and at least six and nine-tenths (6.9) per cent. of copper and aluminum together, the copper and aluminum being present in the 50 ratio of about three parts of copper to about one part of aluminum.

2. An alloy of zinc with copper, aluminum and manganese, said alloy containing 55 about 90 per cent. of zinc and an amount of manganese not less than about 0.25 per cent., and not more than about 4 per cent.

3. An alloy of zinc with copper, aluminum and manganese, said alloy containing zinc, about 6 per cent. of copper, about 2 6 per cent. of aluminum and about 1.5 per cent. of manganese.

In testimony whereof we have signed our names to this specification in the presence of two subscribing witnesses.

HANS GOLDSCHMIDT.

KARL MÜLLER.

Witnesses:

FRANCES M. NUFER,

FREDERICK J. DIETZMAN.